

Dec. 2, 1924.

1,517,675

W. R. HARTUNG

CASTING

Filed March 5, 1921



WITNESSES

*George C. Myers*

INVENTOR

*W. R. HARTUNG*

BY

*Maurice Koo*

ATTORNEYS

## UNITED STATES PATENT OFFICE.

WILLIAM R. HARTUNG, OF CONNELL, WASHINGTON.

## CASTING.

Application filed March 5, 1921. Serial No. 449,850.

*To all whom it may concern:*

Be it known that I, WILLIAM R. HARTUNG, a citizen of United States, and a resident of Connell, in the county of Franklin 5 and State of Washington, have invented certain new and useful Improvements in Castings, of which the following is a specification.

The present invention relates in general 10 to castings and sleeves, and more particularly to a method of chilling, or chilling the interior of castings or chilling sleeves or chilling the interior of cylinders.

In carrying out the invention the mold 15 for the casting or sleeve is first prepared. A dry sand core is coated with graphite and after having been heated in a suitable oven so the sand core is hot it is inserted in the mold. The molten metal is then poured very 20 hot and when the sand core is still hot. Before the core is driven or knocked out it is filled with water from the top of a temperature depending upon the character and depth of the chill desired, cold water being 25 used when it is desired to produce a very substantial depth and relatively hard chill and cold water being used as a lesser degree of these qualities is desired. After the chilling and hardening has been effected by 30 filling or treating the sand core with water from the top, the water being of a temperature corresponding to the effects desired to be produced the core is driven or knocked out and the casting or sleeve is completed.

35 Referring to the accompanying drawing; Figure 1 represents a side elevational view of the core employed in carrying out the present invention; and

40 Figure 2 represents a cross sectional view thereof.

In the drawing the core is designated generally as at *a* and is slightly tapered.

As shown especially in Figure 2 the core 45 is preferably constructed in the main of dry sand designated at *S*, upon the surface of which is applied a coating of graphite, designated at *C*. In carrying out the process the core is adapted after the casting operation proper to receive and contain water 50 with which it is filled from the top to effect the chilling as above described and the slight taper of the core provides for the easy disassembling or disassociation of this element from the casting.

As has been indicated the core is filled 55 with water from the top and is so treated immediately after the metal has been poured for the casting or sleeve.

Make the castings on end and pour the 60 metal very hot.

The sand core is filled with water from the top. When the core is so treated, the water is distributed throughout the sand of the core, whereby a uniform and thorough chill of the casting or sleeve is effected. 65 This method will chill a sleeve of three-fourths of an inch in diameter straight through.

By producing a casting with this method and with a core of this character the interior 70 of castings and the interior or the inside of the cylinders or sleeves are hardened or chilled to any desired degree to provide a better wearing surface and to generally improve the casting or the sleeves. This result 75 is largely effective by reason of the fact that the metal is hardened by the peculiar steps of the process and instrumentalities utilized in connection therewith in such a singular manner that the strength of the casting or sleeve is so enhanced and the metal itself is imparted such a quality as to prolong the life of the casting and to provide 80 a better wearing metal. The process can also be used for cooling the inside or outside 85 of castings to avoid shrinking, cracks, and strains.

I claim:

1. The herein described method of chilling and hardening castings and cylinders 90 and sleeves which consists in preparing a mould and introducing a previously heated and graphite coated sand core therein, pouring the metal while the core is hot and filling the sand core with water of a certain 95 temperature from the top prior to this disassociation of the core from the metal.

2. The herein described method of chilling and hardening the interior of castings and the interior of cylinders and chilling 100 sleeves which consists in filling the sand core with water of a certain temperature from the top prior to disassociation of the sand core from the casting or sleeve all as and for the purposes set forth.

WILLIAM R. HARTUNG.

**Certificate of Correction.**

It is hereby certified that in Letters Patent No. 1,517,675, granted December 2 1924, upon the application of William R. Hartung, Connell, Washington, for an improvement in "Castings," an error appears in the printed specification requiring correction as follows: Page 1, line 27, for the word "cold" read *warm*; and that the said Letters Patent should be read with this correction therein that the same may conform to the record of the case in the Patent Office.

Signed and sealed this 7th day of April, A. D. 1925.

[SEAL.]

**KARL FENNING,**  
*Acting Commissioner of Patents.*